

Aug. 3, 1937.

S. RUBEN

2,088,928

ELECTROLYTIC CONDENSER

Filed Nov. 4, 1935

*Fig. 1*



*Fig. 3*

*Fig. 2*



INVENTOR

*Samuel Ruben*

BY

*Frank Hoblin*

ATTORNEY

## UNITED STATES PATENT OFFICE

2,088,928

## ELECTROLYTIC CONDENSER

Samuel Ruben, New Rochelle, N. Y.

Application November 4, 1935, Serial No. 48,140

8 Claims. (Cl. 175—315)

This invention relates to electrolytic condensers and particularly to electrolytic condensers of "dry" or non-aqueous type.

An object of the invention is to provide an electrolytic condenser having an improved electrolyte.

Another object is the provision of an electrolyte which is viscous, has a high boiling point, a high specific resistance, is hygroscopic, non-corrosive, non-crystalline, which has an organic acid radicle and which is adapted to the production of dry electrolytic condensers by impregnation of the electrolyte into the spacer.

Still another object is the construction of an electrolytic condenser having low leakage and a relatively small amount of deformation when not in use.

A further object is the provision of an electrolytic condenser employing an electrolyte which allows operation on alternating current with a low power factor over a wide operating temperature range.

Other objects will be apparent from the disclosure and the drawing in which:

Fig. 1 is a perspective view, partly broken away, of one embodiment of the invention showing a flat plate condenser;

Fig. 2 is a perspective view of a modification showing the arrangement of the invention in coiled form, and

Fig. 3 is a vertical section of an arrangement somewhat similar to Fig. 2, enclosed within a protective casing.

This invention may be said to be a continuation in part of my co-pending application bearing Serial Number 680,688, filed July 17, 1933.

The present electrolyte differs markedly from the electrolytes of the prior art in its ability to maintain low power factors with specific resistances many times higher than those of the earlier type of materials, such as borates. This is apparently a characteristic associated with the particular ionogen used and is probably due to the fact that the entire electrolyte is the ionization medium, that is to say, there are no inactive or partially active carriers, suspension mediums or fillers.

My invention comprises the use of a lactate of ammonium, potassium or sodium as an improved electrolyte material.

In the dry electrolytic condensers of the prior art, the electrolytes have been essentially compounds and mixtures of a non-aqueous suspension material such as the polyhydric alcohols—glycols and glycerols. The electrolytes produced

were partly compounds of the salts for instance, those salts produced by the combination of boric acid or alkaline base borates with the alcohols, and the conduction was determined by the resulting boiling point as regulated by the residual water content in the electrolyte. As the sparking potential varies with this residual aqueous content, control was naturally established by the boiling point. At some temperatures, these prior electrolytes comprise mixtures of the salt reaction products with the carrier, for example, glycol borates salts dissolved in glycol, so that variations in operating conditions due to changes in operating temperatures were, in part, dependent upon the ratio of compound in solution to the suspension material.

These conditions do not exist in the present electrolyte which is of the non-crystalline type and which is boiled to a temperature higher than that used in the prior art.

I have found that by employing ammonium lactate as the electrolyte, I can produce an electrolytic condenser having a much higher specific resistance than is useable with the borate type and still have a low power factor. For example, it appears that in the construction of an ammonium lactate condenser capable of operation on alternating current, without increase in power factor, when operating at temperatures such as 50° to 60° C., it is very desirable that the electrolyte have a specific resistance in the order of 100,000 ohms per cm.<sup>3</sup> at 20° C. Even with this high resistance, the electrolyte does not require the addition of conductive fillers. This resistance value is obtained by boiling the materials to a temperature in the neighborhood of 195° C.

I prefer to make the electrolyte by the following method: 7.5 c. c. of 28% ammonium hydroxide is added slowly to 10 grams of lactic acid and the solution slowly mixed, to form ammonium lactate. An excess of ammonia can be used as it will be lost on heating. The compound is then boiled to a temperature of 195° C. where it forms a brown viscous and somewhat hygroscopic compound. The boiled electrolyte is more acidic than the original product, thus indicating the presence of a small amount of lactic acid.

While I prefer ammonium lactate, I have also used both sodium and potassium lactate boiled to temperatures such as 150° C. to give adequate resistance values necessary for the proper contact resistance to the formed electrodes. In the formation of an electrolyte employing the sodium hydroxide, I have found that the proportion of

1000 grams of lactic acid to 790 c. c. of a 37½% solution of sodium hydroxide is desirable.

The electrolyte can be readily impregnated into spacers commonly used in dry electrolytic condensers. I have found that a porous grade of paper 4 mils thick is especially suitable in condensers employing the electrolyte of this invention; however, gauze, "cellophane" or other commonly used spacers may also be employed.

10 Alternating current condensers made with this electrolyte are particularly useful as motor starting capacitors operating on 110 volts, the high specific resistance of the electrolyte which reduces the effects of impurities and of leakage variations in plate areas being beneficial for alternating current operation. The electrolyte is also adaptable for use in direct current condensers.

15 The condenser structure used is similar to that now used in the art and is illustrated in the attached drawing in which like numbers indicate like parts.

20 In the flat type condenser of Fig. 1, the two film formed aluminum electrodes 1 and 2 are spaced by the ammonium lactate impregnated 25 spacer 3.

25 In Fig. 2 is shown the condenser of Fig. 1 with the addition of another spacer, 3A, similar to 3, which is necessary in order to prevent shorting of the electrodes.

30 In Fig. 3, the condenser section is housed in metal can 4, having an insulator top 5, through which pass terminals 6 and 7 attached to the respective condenser foils. Insulation at the bottom of the can is provided by pitch 8.

35 Since certain changes in carrying out the construction of the condenser and its components and obvious substitutions can be made in the materials used without departing from the scope of the invention, it is intended that all materials contained in the above description or shown in the accompanying drawing shall be interpreted as illustrative and not in a limiting sense.

40 Having described my invention, what I claim

as new and desire to secure by Letters Patent, is:

1. An electrolytic condenser comprising two electrodes and a contacting conductive medium between the electrodes composed of a lactate of one of the materials ammonium, sodium or potassium. 5

2. An electrolytic condenser comprising two electrodes and an electrolyte of ammonium lactate. 10

3. An electrolytic condenser comprising two electrodes at least one of which is film-forming and a contacting conductive medium between the electrodes composed of ammonium lactate. 15

4. An electrolytic condenser comprising two electrodes at least one of which is film formed and a cellulose spacing medium therebetween permeated substantially entirely with ammonium lactate, said permeated cellulose contacting the electrodes. 20

5. A conductive spacer for electrolytic condensers comprising a flexible cellulose sheet material permeated substantially entirely with ammonium lactate so as to afford a conductive path therethrough. 25

6. An electrolyte for electrolytic condensers composed of a lactate of one of the materials ammonium, postassium and sodium and containing a small amount of lactic acid. 30

7. An electrolytic condenser of the "dry" type 30 comprising a container and a condenser section therein composed of a pair of electrode foils, at least one of which is filmed, a sheet spacer therebetween and a electrolyte held by said spacer composed of ammonium lactate. 35

8. An alternating current capacitor comprising a container and a capacitor section therein composed of a pair of filmed aluminum electrodes, a sheet spacer therebetween and an electrolyte held by said spacer composed of ammonium lactate. 40

SAMUEL RUBEN.